# EUROPEAN PATENT SPECIFICATION

(11) **EP 3 470 556 B1**
(45) Date of publication and mention of the grant of the patent: **10.06.2020**
(21) Application number: 18206666.2
(22) Date of filing: 08.09.2009
(51) Int. Cl.: D01D 5/00

(54) **HIGH THROUGHPUT ELECTROBLOWING PROCESS**
HOCHLEISTUNGSELEKTROBLASVERFAHREN
PROCESSUS DE SOUFFLAGE ÉLECTRIQUE À HAUT RENDEMENT

(30) Priority: 05.09.2008 US 19110208 P
(43) Date of publication of application: 17.04.2019
(62) Divisional of application: 09792294.2
(73) Proprietor: DuPont Safety & Construction, Inc., Wilmington, Delaware 19805 (US)
(72) Inventor: Dee, Gregory T., Wilmington, DE 19802-2652 (US); Hovanec, Joseph Brian, Richmond, VA 23223 (US); Van Meerveld, Jan, 5552 Remich (LU)
(74) Representative: Dannenberger, Oliver Andre

(56) References cited:
- WO-A1-2007/022390
- ZHENG-MING HUANG ET AL: "A review on polymer nanofibers by electrospinning and their applications in nanocomposites", COMPOSITES SCIENCE AND TECHNOLOGY, ELSEVIER, UK, vol. 63, no. 15, 2 July 2003 (2003-07-02), pages 2223-2253, XP002516036, ISSN: 0266-3538 [retrieved on 2003-07-02]

## Description

### CROSS REFERENCE TO RELATED APPLICATIONS

Subject matter disclosed herein may be disclosed and claimed in the following application filed concurrently herewith, assigned to the assignee of the present invention:
"Fiber Spinning Process Using a Weakly Interacting Polymer", Ser. No. 61/191103 (Docket No. TK4955 US PRV), filed in the names of Dee, Hovanec, and VanMeerveld.

### FIELD OF THE INVENTION

The present invention relates to a process for forming a fibrous web from a high throughput electroblowing process.

### BACKGROUND

Solution spinning processes are frequently used to manufacture fibers and nonwoven fabrics, and in some cases have the advantage of high throughputs, such that the fibers or fabrics can be made in large, commercially viable quantities. These processes can be used to make fibrous webs that are useful in medical garments, filters and other end uses that require a selective barrier. The performance of these types of fibrous webs can be enhanced with the utilization of fibers with small diameters.

A type of solution spinning called electroblowing produces very fine fibers by spinning a polymer solution through a spinning nozzle in combination with a blowing gas and in the presence of an electric field.

However, it would be desirable to increase the throughput of this process to increase process efficiencies and lower the cost of manufacturing, without sacrificing fiber uniformity and product quality.

### SUMMARY OF THE INVENTION

The present invention is a fiber spinning process comprising the steps of providing a polymer solution, which comprises at least one polymer dissolved in at least one solvent with a vapor pressure of at least about 6 kPa at 25°C, to a spinneret, issuing the polymer solution in combination with a blowing gas in a direction away from at least one spinning nozzle in the spinneret and in the presence of an electric field wherein the polymer solution is discharged through the spinning nozzle at a discharge rate between about 6 to about 100 ml/min/hole, forming fibers, and collecting the fibers on a collector.

### BRIEF DESCRIPTION OF THE DRAWINGS

The accompanying drawing, which is incorporated in and constitutes a part of this specification, and together with the description, serves to explain the principles of the invention.

Fig. 1 is a schematic of a prior art electroblowing apparatus useful for preparing a fibrous web according to the invention.

### DETAILED DESCRIPTION OF THE INVENTION

The present invention relates to solvent-spun webs and fabrics for a variety of customer end-use applications, such as filtration media, energy storage separators, protective apparel and the like.

The present invention uses an electroblowing process to spin a polymer dissolved in a high vapor pressure solvent at a high rate of throughput into fibers and webs.

The process for making a fiber layer(s) is disclosed in International Publication Number WO2003/080905 (U.S. Serial No. 10/822,325), which is hereby incorporated by reference. Fig. 1 is a schematic diagram of an electroblowing apparatus useful for carrying out the process of the present invention using electroblowing (or "electro-blown spinning") as described in International Publication Number WO2003/080905. This prior art electroblowing method comprises feeding a solution of a polymer in a solvent from a storage tank 100, through a spinneret 102, to a spinning nozzle 104 to which a high voltage is applied, while compressed gas or blowing gas is directed toward the polymer solution through a blowing gas nozzle 106 as the polymer solution exits the spinning nozzle 104 to form fibers, and collecting the fibers into a web on a grounded collector 110 under vacuum created by vacuum chamber 114 and blower 112.

The collection apparatus is preferably a moving collection belt positioned within the electrostatic field between the spinneret 102 and the collector 110. After being collected, the fiber layer is directed to and wound onto a wind-up roll on the downstream side of the collector 110. Optionally, the fibrous web can be deposited onto any of a variety of porous scrim materials arranged on the moving collection belt, such as spunbonded nonwovens, meltblown nonwovens, needle punched nonwovens, woven fabrics, knit fabrics, apertured films, paper and combinations thereof.

Optionally, a secondary gas can contact the fibers downstream from the spinneret to help drive off solvent from the fiber. When electroblowing fibers with a high throughput rate, large quantities of solvent must be removed from the fiber forming polymer solution. The secondary gas can be positioned to impinge the fibers or can be used as a sweeping gas to help remove solvent from the general spinning area.

In order to spin fibers at high throughput or discharge rate, solvents with high vapor pressure can be used. According to the invention, solvents with vapor pressures of at least 6 kPa at 25°C are preferred, of at least 10 kPa at 25°C are more preferred and of at least 20 kPa at 25°C are still more preferred. Suitable solvents with high vapor pressure include methanol (16.9), ethanol (7.9), acetone (30.8), butanone (12.1), dichloromethane (58.1), 1,2-dichloroethane (10.6), trifluoroacetic acid (14.7), ethyl acetate (12.4), tetrahydrofuran (21.6), chloroform (26), carbon tetrachloride (15.4), and hydrocarbons including pentane (68.3), hexane (20.2), heptane (6.1), cyclohexane (13), methylcyclohexane (6.1), and benzene (12.3), where the numbers in parentheses are the vapor pressures of these solvents at 25°C in units of kPa. The vapor pressure data was obtained from "Organic Solvents". Volume 2, fourth edition, by John Riddick, William Bunger, and Theodore Sakano, John Wiley & Sons, 1986 or from the DIPPR® database of physical properties of solvents.

According to the invention, solvents with vapor pressures of at least 6 kPa at 25°C are preferred, of at least 10 kPa at 25°C are more preferred and of at least 20 kPa at 25°C are still more preferred.

The polymer solution can be spun at a temperature of about 0°C to the boiling point of the solvent.

These solvents can be used to prepare polymer solutions that can be spun at a discharge rate between about 6 to about 100 ml/min/hole, more advantageously between about 10 to about 100 ml/min/hole, and most advantageously between about 20 to about 100 ml/min/hole.

The polymer(s) that can be used in making fiber layers in accordance with the process of the present invention are not particularly limited, provided that they are substantially soluble in the selected solvent at the desired concentration and can be spun into fibers by the process described herein. Examples of these polymers generally include hydrocarbon polymers. Examples of hydrocarbon polymers suitable for the present invention include polyolefins, polydienes, polystyrene and blends thereof. Examples polyolefins include polyethylene, polypropylene, poly(1-butene), poly(4-methyl-1-pentene), and blends, mixtures and copolymers thereof.

In addition to the forgoing polymers, other examples include polysulfones, polycarbonates, poly(meth)acrylates, cellulose esters, polyvinylchlorides, and blends thereof. Examples of poly(meth)acrylates include polymethylacrylate and polymethylmethacrylate. Examples of cellulose esters include cellulose triacetate. Examples of polyesters include polyethylene therephthalate, polypropylene therephthalate, polybutylene therephthalate, poly(epsilon-caprolactone), poly(DL-lactic acid) and poly(L-lactide).

The blowing gas can be selected from the group of air, nitrogen, argon, helium, carbon dioxide, hydrocarbons, halocarbons, halohydrocarbons and mixtures thereof. The blowing gas is injected at a flow velocity of about 50 to about 340 m/sec and a temperature from about ambient to about 300°C.

The fibers produced have a number average fiber diameter preferably less than 1,000 nanometers, more preferably less than 800 nanometers and most preferably less than 500 nanometers. The fibers can be continuous or discontinuous. The fibers can have an essentially round cross section shape.

The electric field can have a voltage potential of about 10 to about 100 kV. The electric field can be used to create a corona charge.

The fibers can be collected into a fibrous web comprising round cross section, weakly interacting polymer fibers having a number average fiber diameter less than about 1,000 nanometers.

The secondary gas can be selected from the group of air, nitrogen, argon, helium, carbon dioxide, hydrocarbons, halocarbons, halohydrocarbons and mixtures thereof. The secondary gas is injected at a flow velocity of about 50 to about 340 m/sec and a temperature from about ambient to about 300°C.

### TEST METHODS

Fiber Diameter was determined as follows. Two to three scanning electron microscope (SEM) images were taken of each fine fiber layer sample. The diameter of clearly distinguishable fine fibers were measured from the photographs and recorded. Defects were not included (i.e., lumps of fine fibers, polymer drops, intersections of fine fibers). The number average fiber diameter from about 50 to 300 counts for each sample was calculated.

### EXAMPLES

The fiber examples below were prepared using the general process and apparatus described above with the specific changes as noted below.

### Reference Example 1

A 9 wt% solution of polymethylmethacrylate (PMMA) was dissolved in acetone (vapor pressure of 24.2 kPa at 25°C) at room temperature. A magnetic stirrer was used to agitate the solution. The homogeneous solution was transferred to a sealed glass container and transported to the spin chamber. The solution was transferred into the reservoir of the spin chamber and sealed. A spinneret with a 0.254 mm inside diameter single spinning nozzle was used. A drum collector was used to collect the sample. The spinneret was placed at a negative potential of 100 kV. The collector was grounded. The distance from the spinning nozzle exit to the collector surface was 51 cm. Air was used for the blowing gas. Nitrogen was used for the secondary gas to control the relative humidity and the temperature in the spin chamber. The flow of nitrogen was sufficient to avoid the concentration of the solvent vapor in the spin chamber exceeding the lower explosion limit. The relative humidity was controlled to be less than 11%. The spin chamber temperature was close to 23 °C for the duration of the experiment. A nitrogen pressure of 0.2044 MPa was used to maintain a solution flow rate of 6.7 ml/min/hole. The blowing gas was controlled to maintain an exit velocity on the order of 67 m/sec. The blowing gas temperature was close to 23 °C. Fiber was visible in the plume soon after the solution flow was initiated. Fiber was deposited in a swath on the drum. The number average fiber diameter of the fibers was measured to be 393 nanometers.

### Example 2

A 9 wt% solution of polystyrene was dissolved in dichloromethane (vapor pressure of 58.1 kPa at 25°C) at room temperature. A magnetic stirrer was used to agitate the solution. The homogeneous solution was transferred to a sealed glass container and transported to the spin chamber. The solution was transferred into the reservoir of the spin chamber and sealed. A spinneret with a 0.406 mm inside diameter single spinning nozzle was used. A drum collector was used to collect the sample. The spinneret was placed at a negative potential of 100 kV. The collector was grounded. The distance from the spinning nozzle exit to the collector surface was 95 cm. Air was used for the blowing gas. Air was used for the secondary gas to control the relative humidity and the temperature in the spin chamber. The flow of air was sufficient to avoid the concentration of the solvent vapor in the spin chamber exceeding the lower explosion limit. The relative humidity was controlled to be less than 11%. The spin chamber temperature was close to 32 °C for the duration of the experiment. A nitrogen pressure of 0.515 MPa was used to maintain a solution flow rate of 34.3 ml/min/hole. The blowing gas was controlled to maintain an exit velocity on the order of 150 m/sec. The blowing gas temperature was close to 24 °C. Fiber was visible in the plume soon after the solution flow was initiated. Fiber was deposited in a swath on the drum. The number average fiber diameter of the fibers was measured to be 335 nanometers.

### Example 3

A 9 wt% solution of polystyrene was dissolved in dichloromethane (vapor pressure of 58.1 kPa at 25°C) at room temperature. A magnetic stirrer was used to agitate the solution. The homogeneous solution was transferred to a sealed glass container and transported to the spin chamber. The solution was transferred into the reservoir of the spin chamber and sealed. A spinneret with a 0.406 mm inside diameter single spinning nozzle was used. A drum collector was used to collect the sample. The spinneret was placed at a negative potential of 100 kV. The collector was grounded. The distance from the spinning nozzle exit to the collector surface was 114 cm. Air was used for the blowing gas. Air was used for the secondary gas to control the relative humidity and the temperature in the spin chamber. The flow of air was sufficient to avoid the concentration of the solvent vapor in the spin chamber exceeding the lower explosion limit. The relative humidity was controlled to be less than 11%. The spin chamber temperature was close to 37 °C for the duration of the experiment. A nitrogen pressure of 0.77 MPa was used to maintain a solution flow rate of 57.1 ml/min/hole. The blowing gas was controlled to maintain an exit velocity on the order of 150 m/sec. The blowing gas temperature was close to 24 °C. Fiber was visible in the plume soon after the solution flow was initiated. Fiber was deposited in a swath on the drum. The number average fiber diameter of the fibers was measured to be 630 nanometers.

### Reference Example 4

An 11 wt% solution of Engage 8400 (an ethylene octene copolymer), available from DuPont, was dissolved in methylcyclohexane (vapor pressure of 6.1 kPa at 25°C) using a reflux condenser. A magnetic stirrer was used to agitate the hot solution. The homogeneous solution was transferred to a sealed glass container and transported to the spin chamber. The solution was transferred into the reservoir of the spin chamber and sealed. A spinneret with a 0.4064 mm inside diameter single spinning nozzle was used. A drum collector was used to collect the sample. The spinneret was placed at a negative potential of 100 kV. The collector was grounded. The distance from the spinning nozzle exit to the collector surface was 30 cm. Air was used for the blowing gas. Nitrogen was used for the secondary gas to control the relative humidity and the temperature in the spin chamber. The flow of nitrogen was sufficient to avoid the concentration of the solvent vapor in the spin chamber exceeding the lower explosion limit. The relative humidity was controlled to be less than 9%. The spin chamber temperature was close to 29 °C for the duration of the experiment. A nitrogen pressure of 0.308 MPa was used to maintain a solution flow rate of 12.6 ml/min/hole. The blowing gas was controlled to maintain an exit velocity on the order of 156 m/sec. The blowing gas temperature was close to 28 °C. Once the solution flow was initiated, fiber was visible in the plume. Fiber was deposited in a swath on the drum. The number average fiber diameter of the fibers was measured to be 502 nanometers.

## Claims

1. A fiber spinning process comprising:
providing a polymer solution, which comprises at least one polymer dissolved in at least one solvent with a vapor pressure of at least 6 kPa at 25°C, to a spinneret;
issuing the polymer solution in combination with a blowing gas in a direction away from at least one spinning nozzle in the spinneret and in the presence of an electric field wherein the polymer solution is discharged through the spinning nozzle at a discharge rate between 20 to 100 ml/min/hole;
forming fibers; and
collecting the fibers on a collector.

2. The process according to claim 1, wherein the solvent is selected from the group consisting of methanol, ethanol, acetone, butanone, dichloromethane, 1,2-dichloroethane, trifluoroacetic acid, ethyl acetate, tetrahydrofuran, chloroform, carbon tetrachloride, and hydrocarbons.

3. The process according to claim 2, wherein the hydrocarbons are selected from the group consisting of pentane, hexane, heptane, cyclohexane, methylcyclohexane, and benzene.

4. The process according to any one of claims 1 to 3, wherein the vapor pressure is of at least 10 kPa at 25°C, or alternatively of at least 20 kPa at 25°C.

5. The process according to any one of claims 1 to 4, wherein the blowing gas is selected from the group of air, nitrogen, argon, helium, carbon dioxide, hydrocarbons, halocarbons, halohydrocarbons and mixtures thereof.

6. The process according to any one of claims 1 to 5, wherein the blowing gas is injected at a flow velocity of 50 to 340 m/sec and a temperature from about ambient to 300°C.

7. The process according to any one of claims 1 to 6, wherein the fibers have a number average fiber diameter less than about 1000 nanometers, or alternatively less than 800 nanometers, or alternatively less than 500 nanometers.

8. The process according to any one of claims 1 to 7, wherein the electric field has a voltage potential of 10 kV to 100 kV.

9. The process according to any one of claims 1 to 8, wherein the electrical field is a corona charging field.

10. The process according to any one of claims 1 to 9, wherein the fibers have a cross section shape that is essentially round.

11. The process according to any one of claims 1 to 10, further comprising contacting the fibers with a secondary gas located downstream from the spinneret.

12. The process according to claim 11, wherein the blowing gas is selected from the group of air, nitrogen, argon, helium, carbon dioxide, hydrocarbons, halocarbons, halohydrocarbons and mixtures thereof.

13. The process according to claim 11 or 12, wherein the blowing gas is injected at a flow velocity of 50 to 340 m/sec and a temperature from about ambient to about 300°C.

14. The process according to any one of claims 1 to 13, wherein said at least one polymer in said polymer solution is selected from the group consisting of polyolefins, polydienes, polystyrene, polysulfones, polycarbonates, poly(meth)acrylates, cellulose esters, polyvinylchlorides, polyesters and blends thereof.

15. The process according to claim 14, wherein said at least one polymer in said polymer solution is selected from the group consisting of polyethylene, polypropylene, poly(1-butene), poly(4-methyl-1-pentene) and blends, mixtures and copolymers thereof; polymethylacrylate and polymethylmethacrylate; cellulose triacetate; polyethylene therephthalate, polypropylene therephthalate, polybutylene therephthalate, poly(epsilon-caprolactone), poly(DL-lactic acid) and poly(L-lactide); and blends thereof.

## Patentansprüche

1. Faserspinnverfahren, umfassend:
bereitstellen einer Polymerlösung, die mindestens ein Polymer umfasst, das in mindestens einem Lösemittel mit einem Dampfdruck von mindestens 6 kPa bei 25 °C aufgelöst ist, zu einer Spinndüsenanordnung;
ausgeben der Polymerlösung in Kombination mit einem Gas zum Blasen in einer Richtung weg von mindestens einer Spinndüse in der Spinndüsenanordnung und in Gegenwart eines elektrischen Feldes, wobei die Polymerlösung durch die Spinndüse bei einer Austragsrate zwischen 20 bis 100 ml/min/Loch ausgetragen wird;
ziehen von Fasern; und
aufnehmen der Fasern auf einem Kollektor.

2. Verfahren nach Anspruch 1, wobei das Lösemittel ausgewählt ist aus der Gruppe bestehend aus Methanol, Ethanol, Aceton, Butanon, Dichlormethan, 1,2-Dichlorethan, Trifluoressigsäure, Ethylacetat, Tetrahydrofuran, Chloroform, Tetrachlorkohlenstoff und Kohlenwasserstoffen.

3. Verfahren nach Anspruch 2, wobei die Kohlenwasserstoffe ausgewählt sind aus der Gruppe bestehend aus Pentan, Hexan, Heptan, Cyclohexan, Methylcyclohexan und Benzol.

4. Verfahren nach einem der Ansprüche 1 bis 3, wobei der Dampfdruck mindestens 10 kPa bei 25 °C oder alternativ mindestens 20 kPa bei 25 °C beträgt.

5. Verfahren nach einem der Ansprüche 1 bis 4, wobei das Gas zum Blasen ausgewählt ist aus der Gruppe bestehend aus Luft, Stickstoff, Argon, Helium, Kohlendioxid, Kohlenwasserstoffen, Halogenkohlenstoffen, Halogenkohlenwasserstoffen und Mischungen davon.

6. Verfahren nach einem der Ansprüche 1 bis 5, wobei das Gas zum Blasen eingespritzt wird mit einer Strömungsgeschwindigkeit von 50 bis 340 m/s und einer Temperatur von etwa Umgebungstemperatur bis 300 °C.

7. Verfahren nach einem der Ansprüche 1 bis 6, wobei die Fasern ein Zahlenmittel des Durchmessers von weniger als 1000 Nanometer, oder alternativ weniger als 800 Nanometer oder alternativ weniger als 500 Nanometer aufweisen.

8. Verfahren nach einem der Ansprüche 1 bis 7, wobei das elektrische Feld ein Spannungspotenzial von 10 kV bis 100 kV aufweist.

9. Verfahren nach einem der Ansprüche 1 bis 8, wobei das elektrische Feld ein Coronaladungsfeld ist.

10. Verfahren nach einem der Ansprüche 1 bis 9, wobei die Fasern eine Querschnittform aufweisen, die weitgehend rund ist.

11. Verfahren nach einem der Ansprüche 1 bis 10, ferner umfassend Kontaktieren der Fasern mit einem sekundären Gas, das der Spinndüsenanordnung nachgeschaltet angeordnet ist.

12. Verfahren nach Anspruch 11, wobei das Gas zum Blasen ausgewählt ist aus der Gruppe bestehend aus Luft, Stickstoff, Argon, Helium, Kohlendioxid, Kohlenwasserstoffen, Halogenkohlenstoffen, Halogenkohlenwasserstoffen und Mischungen davon.

13. Verfahren nach Anspruch 11 oder 12, wobei das Gas zum Blasen eingespritzt wird mit einer Strömungsgeschwindigkeit von 50 bis 340 m/s und einer Temperatur von etwa Umgebungstemperatur bis etwa 300 °C.

14. Verfahren nach einem der Ansprüche 1 bis 13, wobei das mindestens eine Polymer in der Polymerlösung ausgewählt ist aus der Gruppe bestehend aus Polyolefinen, Polydienen, Polystyrol, Polysulfonen, Polycarbonaten, Poly(meth)acrylaten, Celluloseestern, Polyvinylchloriden und Mischungen davon.

15. Verfahren nach Anspruch 14, wobei das mindestens eine Polymer in der Polymerlösung ausgewählt ist aus der Gruppe bestehend aus Polyethylenepolypropylen, Poly(1-butene), Poly(4-methyl-1-penten) und Gemischen, Mischungen und Copolymeren davon; Polymethylacrylat und Polymethylmethacrylat; Cellulosetriacetat; Polyethylentherephthalat, Polypropylentherephthalat, Polybutylentherephthalat, Poly(epsilon-caprolacton), Poly(DL-Milchsäure) und Poly(L-Lactid); und Gemischen davon.

## Revendications

1. Procédé de filage de fibres comprenant:
la fourniture d'une solution de polymère, qui comprend au moins un polymère dissous dans au moins un solvant avec une pression de vapeur d'au moins 6 kPa à 25°C, à une filière;
la sortie de la solution de polymère en combinaison avec un gaz soufflant dans une direction s'éloignant d'au moins une buse de filage dans la filière et en présence d'un champ électrique, dans lequel la solution de polymère est déchargée par la buse de filage à un débit de décharge entre 20 et 100 ml/min/trou;
la formation de fibres; et
la récupération des fibres sur un collecteur.

2. Procédé selon la revendication 1, dans lequel le solvant est choisi dans le groupe constitué du méthanol, de l'éthanol, de l'acétone, du butanone, du dichlorométhane, du 1-2-dichloroéthane, de l'acide trifluoroacétique, de l'éthyl acétate, du tétrahydrofurane, du chloroforme, du tétrachloriure de carbone, et des hydrocarbones.

3. Procédé selon la revendication 2, dans lequel les hydrocarbones sont choisis dans le groupe constitué de pentane, hexane, heptane, cyclohexane, méthylcyclohexane et benzène.

4. Procédé selon l'une des revendications 1 à 3, dans lequel la pression de vapeur est d'au moins 10 kPa à 25°C ou alternativement d'au moins 20 kPa à 25°C.

5. Procédé selon l'une des revendications 1 à 4, dans lequel le gaz soufflant est choisi dans le groupe de: air, azote, argon, hélium, dioxyde de carbone, hydrocarbures, halocarbures, halohydrocarbures et mélanges de ceux-ci.

6. Procédé selon l'une des revendications 1 à 5, dans lequel le gaz soufflant est injecté à une vitesse d'écoulement de 50 à 340 m/sec et une température de l'ambiante à 300°C.

7. Procédé selon l'une des revendications 1 à 6, dans lequel les fibres ont un diamètre de fibre moyen en nombre inférieur à 1000 nanomètres, alternativement inférieur à 800 nanomètres, ou alternativement inférieur à 500 nanomètres.

8. Procédé selon l'une des revendications 1 à 7, dans lequel le champ électrique a un potentiel de tension de 10 kV à 100 kV.

9. Procédé selon l'une des revendications 1 à 8, dans lequel le champ électrique est un champ à chargement couronne.

10. Procédé selon l'une des revendications 1 à 9, dans lequel les fibres ont une forme de section transversale qui est essentiellement ronde.

11. Procédé selon l'une des revendications 1 à 10, comprenant en outre la mise en contact des fibres avec un gaz secondaire localisé en aval de la filière.

12. Procédé selon la revendication 11, dans lequel le gaz soufflant est choisi dans le groupe de : aire, azote, argon, hélium, dioxyde de carbone, hydrocarbures, halocarbures, halohydrocarbures et mélanges de ceux-ci.

13. Procédé selon la revendication 11 ou 12, dans lequel le gaz soufflant est injecté à une vitesse d'écoulement de 50 à 340 m/sec et une température d'environ l'ambiante à environ 300°C.

14. Procédé selon l'une des revendications 1 à 13, dans lequel ledit au moins un polymère dans ladite solution de polymère est choisi dans le groupe constitué de: polyoléfines, polydiènes, polystyrène, polysulfones, polycarbonates, poly(méth)acrylates, esters de cellulose, polyvinylchlorures et mixtures de ceux-ci.

15. Procédé selon la revendication 14, dans lequel ledit au moins un polymère dans ladite solution de polymère est choisi dans le groupe constitué de: polyéthylène polypropylène, poly(1-butène), poly(4-méthyl-1-pentène) et des mixtures, des mélanges et copolymères de ceux-ci ; polyméthylacrylate et polyméthylméthacrylate ; triacétate de cellulose ; polyéthylène téréphtalate, polypropylène théréphthalate ; polybutilène théréphthalate, poly(epsilon-caprolactone), poly(DL-acide lactique) et poly(L-lactide) ; et des mixtures de ceux-ci.
